

# United States Patent Office

2,781,305

Patented Feb. 12, 1957

1

2,781,305

## ELECTRODEPOSITION OF NICKEL

Henry Brown, Huntington Woods, Mich., assignor to The Udylite Research Corporation, Detroit, Mich., a corporation of Michigan

No Drawing. Application August 14, 1953,  
Serial No. 374,418

14 Claims. (Cl. 204—49)

This invention relates to the electrodeposition of nickel from an aqueous acidic bath.

One object of this invention is to decrease the grain size and increase the luster of the nickel deposit.

A second and major object is the electrodeposition of brilliant, highly lustrous, ductile nickel plate.

It has been found that these objects can be accomplished by the use of certain organic compounds in the aqueous acidic nickel baths.

The first object mentioned above can be accomplished by the addition to the Watt's type of nickel bath or its modifications of certain amides carrying an unsaturated olefinic group. The presence of these particular amides, which are more specifically illustrated by the compounds set forth in Table III, may be designated generally by Formula A.

### FORMULA A



where  $R_1$  and  $R_2$  are selected from the group consisting of hydrogen, acetyl, chlorine, bromine, methyl, methyl carboxy, carbonyl, carboxy and aldehydo, phenyl and furyl and the chloro, bromo, acetyl, methyl, carboxy, amino, methoxy, ethoxy, dioxymethylene, carbonyl amido, hydroxy and ethyl substitution products of phenyl and furyl,  $R_3$  and  $R_4$  are selected from the group consisting of hydrogen, methyl, formyl, acetyl, amino, amido, imido, carboxy, carbonyl, benzoyl and nicotinoyl radicals. The types of compounds which are encompassed by Formula A are illustrated in the compounds designated A, B, C and D.

### COMPOUND A

When  $R_1$ ,  $R_2$ ,  $R_3$  and  $R_4$  are hydrogen, we have



### COMPOUND B

When  $R_1$  is a phenyl,  $R_2$ ,  $R_3$  and  $R_4$  are hydrogen, we have



### COMPOUND C

When  $R_1$  is methyl carboxy,  $R_2$ ,  $R_3$  and  $R_4$  are hydrogen, we have



Monomethyl maleic acid monoamide (methyl ester of maleamic acid)

2

### COMPOUND D

When  $R_1$  is carbonyl,  $R_2$  and  $R_3$  are chlorine and  $R_4$  is hydrogen, we have



### Mucochloric acid amide

The presence of the compounds represented by Formula A in the bath causes the nickel plate which is electrodeposited therefrom to be very fine-grained (even though cloudy and milky in appearance), and to show marked increasing luster with continued plating.

It was further found that the second object, the production of brilliant, highly lustrous, ductile nickel plate, could be accomplished by the use in conjunction with the compounds represented by Formula A, of a material containing another and different functional group, namely, the unsaturated methylene sulfone group,  $=C-SO_2$ , as exemplified by benzene sulfonamides and sulfonimides. The presence of a compound represented by Formula A alone in a Watt's type nickel bath, or the presence of a material containing the unsaturated methylene sulfone group alone, gives no obvious indication of the remarkably different and enhanced result which occurs when both materials are concurrently present.

While the simpler aryl sulfonamides and some of the aryl sulfonic acids produce bright and mirror-like deposits on buffed metals such as buffed brass, these compounds fail to accomplish the same result on steel which is polished, for example, with 200 emery paper or where the nickel is plated on top of matte (but unburnt) copper plate of 0.003" to 0.0005" thickness, and yield in these cases plate of dull and grey appearance. If, however, the compound represented by Formula A and a material containing the unsaturated methylene sulfone group are used together, a brilliant mirror-like deposit can be obtained even on a matte copper deposit.

The aryl sulfones (sulfonamides, sulfonic acids) in general do not have a critical concentration range in the bath, and they produce practically no further improvement after their optimum concentration is attained. In the case of a compound represented by Formula A, it is thought that a mechanism of the functioning in a Watt's type nickel bath comprises a preferential reduction of the unsaturated compound with respect to the nickel ion, whereas with the aryl sulfones, the nickel ion is reduced preferentially. The variation of the reduction with the variation of the potentials between adjacent high and low points will account for the rate of brightening, or "smoothing out" effect.

The uniqueness of the aryl sulfones, or broadly the



compounds, seems to be mainly tied up with the rate of reduction of the positive valent sulfur compound to negative valent sulfur compound, and the mechanism of its deposition. The fact that with  $\alpha$ -naphthalene sulfonamide as the only organic compound in the bath, not only is the odor of naphthalene apparent at the cathode during the plating, but also the analysis of the plate shows the presence of carbon as well as sulfur, and this indicates that the mechanism of the reduction is not of the simplest form.

It is not the sulfone group alone that is responsible for the effect of the aryl sulfones because the saturated alkyl sulfones are not nearly as effective as the aryl sulfones. The benzene and toluene sulfonamides and ortho benzoyl sulfonimide are more effective than aryl monosulfonic acids, especially of the benzene series,

nevertheless, the latter, even though they may not produce bright plate on buffed metals, will give brilliant ductile plate when used in combination with a compound represented by Formula A.

The concentration of a compound represented by Formula A or a mixture thereof which may be advantageously employed is not critical in any concentration up to saturation, and may be used at concentrations between about 0.1 to about 2.0 grams/liter, the preferred concentration being .6-1.2 grams/liter.

In keeping with their chemical activity, the higher the temperature of the bath, the more active are the unsaturated groups in the bath and smaller concentrations of compounds carrying them must be used. Furthermore, they function best at the higher pH values of the nickel bath, that is, 3.0 to 5.2, and their effectiveness in most cases drops rather suddenly when the pH is lowered past a certain value (in general, at a pH below 3.0 or 2.5, depending on the type of unsaturated compound and on the temperature). The lower the temperature, the higher are the pH values that should be used, and conversely.

The best cathode film buffer is boric acid and it is important to keep its concentration high (over 30 grams/liter), especially in the warm baths. Other buffers may be used in small amount (1 to 5 grams/liter) with the boric acid with beneficial effects, such as formic, citric, fluoboric acids, etc., but they are not recommended to be used alone.

In the use of a compound represented by Formula A alone in the bath, or in the presence of the aryl sulfones, ammonium salts should be kept at a minimum. A concentration of zinc and copper ions in the bath should also be kept as low as possible. This is especially desirable where the concentration of aryl sulfones are low in the bath or the latter compounds are absent.

The baths may be operated at pH values ranging from 2.0 to 5.5 and temperatures ranging from 20° C. to 70° C., and the preferred current density ranges may be from 5 to 150 amps./sq. ft., depending on the agitation, the temperature of the bath and the concentration and the type of nickel salts. The benzene sulfonamides and sulfonimides may be used effectively in concentrations of from 0.05 gram/liter to saturation.

In Table I are listed preferred bath compositions.

Table I

| NISO <sub>4</sub> H <sub>2</sub> O,<br>g/l. | NiCl <sub>2</sub> ,<br>6H <sub>2</sub> O,<br>g/l. | H <sub>3</sub> BO <sub>3</sub> ,<br>g/l. | Ni(BF <sub>4</sub> ) <sub>2</sub> ,<br>g/l. | Temp.<br>(° C.) | Optimum<br>pH |
|---------------------------------------------|---------------------------------------------------|------------------------------------------|---------------------------------------------|-----------------|---------------|
| 250-300                                     | 35-75                                             | 35-40                                    | -----                                       | 40-65           | 2.5-4.5       |
| 100-300                                     | 35-40                                             | 35-40                                    | -----                                       | 40-65           | 2.5-4.5       |
| 75-100                                      | 200-250                                           | 35-40                                    | -----                                       | 40-65           | 2.5-4.5       |
| 200-250                                     | 30-60                                             | 35-40                                    | 7-15                                        | 40-50           | 2.8-5.0       |
| -----                                       | 0-35                                              | 0-40                                     | 150-300                                     | 40-50           | 2.8-5.0       |

In Table II are listed representative examples of organic sulfonamides, sulfonimides and sulfonic acids which may be employed in conjunction with the addition agents represented by Formula A and typified in Table III.

Table II

| Sulfur-containing brighteners:                | Optimum conc.<br>grams/liter |
|-----------------------------------------------|------------------------------|
| 1. Benzene sulfonamide                        | 0.1-3                        |
| 2. Toluene sulfonamides (o- and p-)           | 0.1-2                        |
| 3. o-Benzoyl sulfimide                        | 0.1-2                        |
| 4. N-benzoyl benzene sulfonimide              | 0.1-1                        |
| 5. p-Toluene sulfonchloramide                 | 0.1-1                        |
| 6. p-Brom benzene sulfonamide                 | 0.1-1                        |
| 7. 6-chlor o-benzoyl sulfimide                | 0.1-1                        |
| 8. m-Aldehydo benzene sulfonamide             | 0.1-1                        |
| 9. Sulfomethyl benzene sulfonamide            | 0.1-6                        |
| 10. Benzene sulfonamide m-carboxylic<br>amide | 0.1-3                        |

| 4                                                      |       |
|--------------------------------------------------------|-------|
| 11. 7-aldehydo o-benzoyl sulfimide                     | 0.1-3 |
| 12. N-acetyl benzene sulfonimide                       | 0.1-2 |
| 13. Methoxy benzene sulfonamides                       | 0.1-1 |
| 14. Hydroxymethyl benzene sulfonamide                  | 0.1-2 |
| 15. Vinyl sulfonamide                                  | 4-12  |
| 16. Allyl sulfonamide                                  | 4-12  |
| 17. Benzene sulfonic acids (mono-, di, and<br>tri-)    | 1-15  |
| 18. p-Brom benzene sulfonic acid                       | 3-6   |
| 19. Benzaldehyde sulfonic acids (o, m, p-)             | 2-6   |
| 20. Diphenyl sulfone sulfonic acid                     | 1-8   |
| 21. Naphthalene sulfonic acids (mono- di,<br>and tri-) | 1-8   |
| 22. Benzene sulfohydroxamic acid                       | 1-5   |
| 23. p-Chlor benzene sulfonic acid                      | 1-5   |
| 24. Diphenyl sulfonic acid                             | 1-5   |
| 25. m-Diphenyl benzene sulfonic acid                   | 1-4   |
| 26. 2-chloro-5-sulfobenzaldehyde                       | 1-5   |
| 27. m-Benzene disulfonamide                            | 0.5-1 |
| 28. Allyl sulfonic acid                                | 4-12  |
| 29. Cinnamyl sulfonic acid                             | 0.1-8 |
| 30. Cinnamyl sulfonamide                               | 0.1-3 |

In Table III are listed representative examples of specific compounds which are covered by Formula A and are suitable for the purposes of this invention, when used alone in a Watt's type nickel bath or in combination with organic sulfonamides, sulfonimides and sulfonic acids of Table II.

Table III

| Compound<br>No. | Unsaturated amides                                                       | Optimum<br>Conc.,<br>grams/<br>liter |
|-----------------|--------------------------------------------------------------------------|--------------------------------------|
| 1.              | Acrylamide                                                               | 0.1-1.2                              |
| 2.              | N-acetyl acrylamide                                                      | 0.1-1.2                              |
| 3.              | Cinnamic amide                                                           | 0.1-1.2                              |
| 4.              | o-Chlorocinnamic amide                                                   | 0.1-1.2                              |
| 5.              | p-Chloroacrylamide                                                       | 0.1-1.2                              |
| 6.              | 2-furanacrylamide                                                        | 0.1-1.2                              |
| 7.              | p-Methoxycinnamic amide                                                  | 0.1-1.2                              |
| 8.              | Methacrylamide                                                           | 0.1-1.2                              |
| 9.              | N-acetyl acrylamide                                                      | 0.1-1.2                              |
| 10.             | Fumaramide (di-amide)                                                    | 0.1-1.2                              |
| 11.             | Chlorofumaramide                                                         | 0.1-1.2                              |
| 12.             | Chloromaleic amide                                                       | 0.1-1.2                              |
| 13.             | Maleic imide                                                             | 0.1-1.2                              |
| 14.             | Phenyl maleic imide                                                      | 0.1-1.2                              |
| 15.             | N-phenyl maleic imide                                                    | 0.1-1.2                              |
| 16.             | α, β-Di-phenyl maleic imide                                              | 0.1-1.2                              |
| 17.             | α, β-Di-phenyl maleic amide (di-amide)                                   | 0.1-1.2                              |
| 18.             | N-nicotinoyl acrylamide                                                  | 0.1-1.2                              |
| 19.             | N-allyl acrylamide                                                       | 0.1-1.2                              |
| 20.             | Maleic acid hydrazide                                                    | 0.1-1.2                              |
| 21.             | N-methyl acrylamide                                                      | 0.1-1.2                              |
| 22.             | N-benzoyl acrylamide                                                     | 0.1-1.2                              |
| 23.             | Atropyl amide                                                            | 0.1-1.2                              |
| 24.             | Mucochloric acid amide                                                   | 0.1-1.2                              |
| 25.             | Mucobromic acid amide                                                    | 0.1-1.2                              |
| 26.             | N-tert, butyacrylamide                                                   | 0.1-1.2                              |
| 27.             | N-acryloylurea                                                           | 0.1-1.2                              |
| 28.             | β-Piperonylacrylamide                                                    | 0.1-1.2                              |
| 29.             | o-Hydroxy cinnamic amide                                                 | 0.1-1.2                              |
| 30.             | o-Methoxy cinnamic amide                                                 | 0.1-1.2                              |
| 31.             | p-Carbonyl-amide cinnamic amide (p-Carbonyl-<br>amide phenyl acrylamide) | 0.1-1.2                              |
| 32.             | o-Acetyl cinnamic amide                                                  | 0.1-1.2                              |
| 33.             | Mono 2-methoxyethyl maleic acid monoamide                                | 0.1-1.2                              |

Although Table III shows the optimum concentration of the compounds therein listed to be between 0.1 and 1.2 grams/liter, these compounds may be used in concentrations up to saturation, especially when used in conjunction with benzene sulfonamides, toluene sulfonamides and o-benzoyl sulfimide. In general, a concentration higher than about 2.5 grams per liter is unnecessary.

It will be understood that any of the compounds listed in Table III may be used separately in a Watt's type nickel bath or in combination with any of the organic sulfonamides, sulfonimides or sulfonic acids of Table II in any of the typical baths set forth in Table I. For purposes of further illustration, the examples given below set forth certain preferred embodiments of the invention.

5  
EXAMPLE I

|                                           | Grams/liter |
|-------------------------------------------|-------------|
| $\text{NiSO}_4 \cdot 6\text{H}_2\text{O}$ | 250-300     |
| $\text{NiCl}_2 \cdot 6\text{H}_2\text{O}$ | 60          |
| $\text{H}_3\text{BO}_3$                   | 45          |
| Acrylamide                                | 1.0-1.8     |
| Benzene sulfonamide                       | 0.5-3       |

## EXAMPLE II

|                                           | Grams/liter |
|-------------------------------------------|-------------|
| $\text{NiSO}_4 \cdot 6\text{H}_2\text{O}$ | 250-300     |
| $\text{NiCl}_2 \cdot 6\text{H}_2\text{O}$ | 40-60       |
| $\text{H}_3\text{BO}_3$                   | 40-50       |
| Cinnamic amide                            | 0.6-1.2     |
| Benzene sulfonamide                       | 0.5-3       |

## EXAMPLE III

|                                           | Grams/liter |
|-------------------------------------------|-------------|
| $\text{NiSO}_4 \cdot 6\text{H}_2\text{O}$ | 50          |
| $\text{NiCl}_2 \cdot 6\text{H}_2\text{O}$ | 250         |
| $\text{H}_3\text{BO}_3$                   | 40-50       |
| 2-furanacrylamide                         | 0.8         |
| o-Benzoyl sulfimide                       | 1-2         |
| o- or p-Toluene sulfonamide               | 1-3         |

## EXAMPLE IV

|                            | Grams/liter |
|----------------------------|-------------|
| $\text{Ni}(\text{BF}_4)_2$ | 100-200     |
| $\text{H}_3\text{BO}_3$    | 30          |
| Fumaramide                 | 1.0-1.5     |
| o-Benzoyl sulfimide        | 1-2         |
| <sup>1</sup> (Sat.)        |             |

The addition agents of this invention may consist of a compound or mixture of compounds represented by Formula A as such, or may consist of an admixture of at least one compound represented by Formula A and at least one compound selected from the group consisting of organic sulfonamides, sulfonimides and sulfonic acids.

This application is a continuation-in-part of my prior application, Serial No. 749,344, filed May 20, 1947, which was itself a continuation-in-part of my prior application, Serial No. 366,385, filed November 20, 1940, both of which are now abandoned.

What is claimed is:

1. A bath for electrodepositing fine-grained lustrous nickel comprising an aqueous acidic nickel solution consisting essentially of at least one material selected from the group consisting of nickel sulfate, nickel chloride and nickel fluoborate, having dissolved therein at least one brightener selected from the group consisting of organic sulfonamides, sulfonimides and sulfonic acids, and additionally a minor amount of a compound having the formula



where  $\text{R}_1$  and  $\text{R}_2$  are selected from the group consisting of hydrogen, chlorine, bromine, methyl, methyl carboxy, carbonyl, carboxy, aldehydo, phenyl, furyl and the chloro, bromo, acetyl, methyl, carboxy, amino, methoxy, ethoxy, dioxyethylene, carbonyl amido, hydroxy and ethyl substitution products of phenyl and furyl,  $\text{R}_3$  and  $\text{R}_4$  are selected from the group consisting of hydrogen, methyl, formyl, acetyl, amino, amido, imido, carboxy, carbonyl, benzoyl and nicotinoyl radicals.

2. A bath for electrodepositing bright nickel comprising an aqueous acidic nickel solution consisting essentially of at least one nickel salt selected from the group consisting of nickel sulfate, nickel chloride and nickel fluoborate, having dissolved therein about 0.1 gram per liter to saturation of at least one brightener selected from the group consisting of organic sulfonamides, sulfonimides, and sulfonic acids, and about 0.1 gram per liter to saturation of a compound having the formula



where  $\text{R}_1$  and  $\text{R}_2$  are selected from the group consisting of hydrogen, chlorine, bromine, methyl, methyl carboxy, carbonyl, carboxy, aldehydo, phenyl, furyl and the chloro, bromo, acetyl, methyl, carboxy, amino, methoxy, ethoxy, dioxyethylene, carbonyl amido, hydroxy and ethyl substitution products of phenyl and furyl,  $\text{R}_3$  and  $\text{R}_4$  are selected from the group consisting of hydrogen, methyl, formyl, acetyl, amino, amido, imido, carboxy, carbonyl, benzoyl and nicotinoyl radicals.

3. A method for electrodepositing nickel to obtain bright nickel comprising the step of electrodepositing nickel from an aqueous acidic nickel solution consisting essentially of at least one material selected from the group consisting of nickel sulfate, nickel chloride and nickel fluoborate, in the presence of at least one brightener selected from the group consisting of organic sulfonamides, sulfonimides and sulfonic acids and additionally a minor amount of a compound soluble in the said acid nickel solution having the formula



where  $\text{R}_1$  and  $\text{R}_2$  are selected from the group consisting of hydrogen, chlorine, bromine, methyl, methyl carboxy, carbonyl, carboxy, aldehydo, phenyl, furyl and the chloro, bromo, acetyl, methyl, carboxy, amino, methoxy, ethoxy, dioxyethylene, carbonyl amido, hydroxy and ethyl substitution products of phenyl and furyl,  $\text{R}_3$  and  $\text{R}_4$  are selected from the group consisting of hydrogen, methyl, formyl, acetyl, amino, amido, imido, carboxy, carbonyl, benzoyl and nicotinoyl radicals.

4. A method for electrodepositing nickel to obtain bright nickel comprising the step of electrodepositing nickel from an aqueous acidic nickel solution consisting essentially of at least one material selected from the group consisting of nickel sulfate, nickel chloride and nickel fluoborate, in the presence of about 0.1 gram per liter to saturation of at least one brightener selected from the group consisting of organic sulfonamides, sulfonimides and sulfonic acids, and about 0.1 gram per liter to saturation of at least one compound soluble in the said acid nickel solution having the formula



where  $\text{R}_1$  and  $\text{R}_2$  are selected from the group consisting of hydrogen, chlorine, bromine, methyl, methyl carboxy, carbonyl, carboxy, aldehydo, phenyl, furyl and the chloro, bromo, acetyl, methyl, carboxy, amino, methoxy, ethoxy, dioxyethylene, carbonyl amido, hydroxy and ethyl substitution products of phenyl and furyl,  $\text{R}_3$  and  $\text{R}_4$  are selected from the group consisting of hydrogen, methyl, formyl, acetyl, amino, amido, imido, carboxy, carbonyl, benzoyl and nicotinoyl radicals.

5. A bath in accordance with claim 1 wherein the unsaturated amide is cinnamic amide and is present in an amount of about 0.1 to 1.2 grams/liter.

6. A bath in accordance with claim 1 wherein said unsaturated amide is o-chlorocinnamic amide and is present in an amount of about 0.1 to 1.2 grams/liter.

7. A bath in accordance with claim 1 wherein said unsaturated amide is mucochloric acid amide and is present in an amount of about 0.1 to 1.2 grams/liter.

8. A bath in accordance with claim 1 wherein said unsaturated amide is acrylamide and is present in an amount of about 0.1 to 1.2 grams/liter.

9. A bath in accordance with claim 1 wherein said unsaturated amide is N-methyl acrylamide and is present in an amount of about 0.1 to 1.2 grams/liter.

10. A method in accordance with claim 3 wherein said unsaturated amide is cinnamic amide and is present in an amount of about 0.1 to 1.2 grams/liter.

11. A method in accordance with claim 3 wherein said unsaturated amide is o-chlorocinnamic amide and is present in an amount of about 0.1 to 1.2 grams/liter.

12. A method in accordance with claim 3 wherein said unsaturated amide is mucochloric acid amide and is present in an amount of about 0.1 to 1.2 grams/liter.

13. A method in accordance with claim 3 wherein said unsaturated amide is acrylamide and is present in an amount of about 0.1 to 1.2 grams/liter.

14. A method in accordance with claim 3 wherein said unsaturated amide is N-methyl acrylamide and is present in an amount of about 0.1 to 1.2 grams/liter.

References Cited in the file of this patent

UNITED STATES PATENTS

2,648,627 Donnelly \_\_\_\_\_ Aug. 11, 1953

OTHER REFERENCES

Raub et al.: Metal Finishing, June 1940, pp. 315-316.